



US011591748B2

(12) **United States Patent**  
**Gigrich**

(10) **Patent No.:** **US 11,591,748 B2**  
(45) **Date of Patent:** **Feb. 28, 2023**

(54) **HEAT TREATED MULTILAYER KNITTED TEXTILE OF LIQUID CRYSTAL POLYMER FIBERS AND MODIFIED POLYACRYLONITRILE FIBERS, AND PROCESS FOR MAKING SAME**

(71) Applicant: **Shadow Works, LLC**, Lorton, VA (US)

(72) Inventor: **James Gigrich**, Lorton, VA (US)

(73) Assignee: **SHADOW WORKS, LLC**, Lorton, VA (US)

(\*) Notice: Subject to any disclaimer, the term of this patent is extended or adjusted under 35 U.S.C. 154(b) by 198 days.

(21) Appl. No.: **17/200,879**

(22) Filed: **Mar. 14, 2021**

(65) **Prior Publication Data**

US 2021/0292967 A1 Sep. 23, 2021

**Related U.S. Application Data**

(60) Provisional application No. 62/960,701, filed on Jan. 14, 2020.

(51) **Int. Cl.**

**D06P 5/00** (2006.01)  
**D06P 1/52** (2006.01)  
**D01D 5/00** (2006.01)  
**D02G 3/04** (2006.01)  
**D02G 3/22** (2006.01)  
**D02G 3/44** (2006.01)  
**D06P 5/20** (2006.01)

(52) **U.S. Cl.**

CPC ..... **D06P 1/5271** (2013.01); **D01D 5/0023** (2013.01); **D02G 3/045** (2013.01); **D02G 3/047** (2013.01); **D02G 3/22** (2013.01); **D02G 3/443** (2013.01); **D06P 5/2066** (2013.01)

(58) **Field of Classification Search**

CPC .... D06P 1/5271; D06P 5/2066; D06P 3/8233; D06P 5/2011; D06P 5/2083; D06P 3/8204; D01D 5/0023; D02G 3/045; D02G 3/047; D02G 3/22; D02G 3/443; D06C 7/02; D01F 6/625; D01F 6/84 USPC ..... 8/494 See application file for complete search history.

(56)

**References Cited**

U.S. PATENT DOCUMENTS

2,025,175 A 12/1935 Pearsall  
2,200,134 A 5/1940 Schlack  
2,460,206 A 1/1949 Wentz  
2,685,120 A 8/1954 Brant

(Continued)

FOREIGN PATENT DOCUMENTS

CN 103233317 A \* 8/2013 ..... D06P 3/54  
CN 107964808 A \* 4/2018 ..... D01F 2/06  
CN 110678594 A \* 1/2020 ..... B32B 5/0267

*Primary Examiner* — Eisa B Elhilo

(74) *Attorney, Agent, or Firm* — Juneau & Mitchell; Todd L. Juneau

(57) **ABSTRACT**

The invention relates to a process for manufacturing a multilayer knitted textile by heating a multi-layer knitted textile in the presence of one or more dye compounds, wherein the multilayer knitted textile comprises a fabric outer layer and a fabric inner layer, wherein the fabric outer layer is knit from a first yarn containing a combination of modacrylic fibers and cotton fibers, wherein the fabric inner layer is knit from a second yarn made from 50-90% HBA/HNA filaments, wherein the heating shrinks the outer layer from about 5 to 25% in length, width, or both.

**20 Claims, 14 Drawing Sheets**

A multilayer article comprising knitted textiles assembled to form the multilayer article that is abrasion resistant, penetration resistant, laceration resistant, and flame resistant  
said multilayer article having a  
(i) HEAT-TIGHTENED OUTER LAYER comprising a flame resistant, knitted textile made of a first yarn containing modacrylic, cotton and optionally FR rayon, Opan, or aramid fibers; and  
(ii) an INNER LAYER comprising a penetration resistant, knitted textile made of a second yarn made from 50-90% HBA/HNA filaments;  
wherein the multilayer article is optionally subjected to heat treatment to obtain shrinkage.

| (56)                  | References Cited |                    |                 |         |                                       |
|-----------------------|------------------|--------------------|-----------------|---------|---------------------------------------|
| U.S. PATENT DOCUMENTS |                  |                    |                 |         |                                       |
| 3,157,982 A           | 11/1964          | Alexandre          | 5,902,355 A     | 5/1999  | Kurahasi et al.                       |
| 3,173,189 A           | 3/1965           | Lacy               | 6,140,261 A     | 10/2000 | Uhlmann                               |
| 3,241,906 A           | 3/1966           | Smith et al.       | 6,521,000 B1    | 2/2003  | McFarland et al.                      |
| 3,247,569 A           | 4/1966           | Gliksmann et al.   | 6,620,212 B1    | 9/2003  | Handermann et al.                     |
| 3,263,458 A           | 8/1966           | Cohn et al.        | 6,689,461 B2    | 2/2004  | Koyanagi et al.                       |
| 3,281,205 A           | 10/1966          | Runton             | 6,848,151 B2    | 2/2005  | Bakker et al.                         |
| 3,289,401 A           | 12/1966          | Gliksmann et al.   | 6,861,093 B2    | 3/2005  | Klutz et al.                          |
| 3,310,857 A           | 3/1967           | Loftin et al.      | 6,869,679 B1    | 3/2005  | Negola                                |
| 3,367,150 A           | 2/1968           | Smith et al.       | 7,141,075 B1    | 11/2006 | Stackhouse et al.                     |
| 3,403,433 A           | 10/1968          | Schoeneberg        | 7,674,301 B2    | 3/2010  | Brown et al.                          |
| 3,414,957 A           | 12/1968          | Langstaff et al.   | 7,943,536 B2    | 5/2011  | D'Ottaviano                           |
| 3,481,685 A           | 12/1969          | White              | 8,060,963 B2    | 11/2011 | Ronchi                                |
| 3,498,737 A           | 3/1970           | Reeves et al.      | 8,187,342 B2    | 5/2012  | Oswal et al.                          |
| 3,571,871 A           | 3/1971           | Caroselli et al.   | 8,375,537 B2    | 2/2013  | Liu et al.                            |
| 3,602,966 A           | 9/1971           | Fleissner          | 9,181,652 B2    | 11/2015 | Harrison                              |
| 3,619,103 A           | 11/1971          | Williams et al.    | 9,677,206 B2    | 6/2017  | Lee et al.                            |
| 3,628,224 A           | 12/1971          | Murotani et al.    | 9,689,092 B2    | 6/2017  | Liao et al.                           |
| 3,653,801 A           | 4/1972           | Du Pont            | 9,702,064 B2    | 7/2017  | Goenka et al.                         |
| 3,852,948 A           | 12/1974          | Ruddell et al.     | 10,119,207 B2   | 11/2018 | Casanova Royo                         |
| 3,871,819 A           | 3/1975           | Greer              | 10,196,763 B2   | 2/2019  | Debnath et al.                        |
| 3,876,370 A           | 4/1975           | Birke et al.       | 10,422,055 B2 * | 9/2019  | Sytz ..... D02G 3/44                  |
| 3,895,909 A           | 7/1975           | Greer              | 10,793,984 B2   | 10/2020 | Ballone et al.                        |
| 3,906,755 A           | 9/1975           | Sando et al.       | 2002/0133888 A1 | 9/2002  | Boyes                                 |
| 3,927,971 A           | 12/1975          | Meier Windhorst    | 2003/0221301 A1 | 12/2003 | Marg et al.                           |
| 3,986,824 A           | 10/1976          | Waibel et al.      | 2005/0060820 A1 | 3/2005  | Lunsford et al.                       |
| 4,046,506 A           | 9/1977           | Feeess et al.      | 2005/0124245 A1 | 6/2005  | Liao                                  |
| 4,056,354 A           | 11/1977          | Pittman et al.     | 2005/0132509 A1 | 6/2005  | Chuang et al.                         |
| 4,086,112 A           | 4/1978           | Porter             | 2005/0217037 A1 | 10/2005 | Negola                                |
| 4,101,270 A           | 7/1978           | Fleissner          | 2006/0037154 A1 | 2/2006  | Goineau et al.                        |
| 4,215,991 A           | 8/1980           | Steiger            | 2006/0096073 A1 | 5/2006  | Stoppa et al.                         |
| 4,240,790 A           | 12/1980          | von der Eltz       | 2006/0225226 A1 | 10/2006 | Merikoski                             |
| 4,256,684 A           | 3/1981           | Achard et al.      | 2007/0000066 A1 | 1/2007  | Chuang et al.                         |
| 4,260,389 A           | 4/1981           | Lister             | 2007/0259583 A1 | 11/2007 | Laycock et al.                        |
| 4,280,496 A           | 7/1981           | Lister             | 2008/0010793 A1 | 1/2008  | Wildeman                              |
| 4,299,015 A           | 11/1981          | Marcus et al.      | 2008/0115289 A1 | 5/2008  | Stackhouse                            |
| 4,342,565 A           | 8/1982           | Teague et al.      | 2009/0191777 A1 | 7/2009  | Liao                                  |
| 4,447,489 A           | 5/1984           | Linhart et al.     | 2009/0211894 A1 | 8/2009  | Ribeiro De Almeida Carneiro Pa et al. |
| 4,452,607 A           | 6/1984           | Wessely            | 2013/0269123 A1 | 10/2013 | Liu et al.                            |
| 4,517,715 A           | 5/1985           | Yoshida et al.     | 2014/0053348 A1 | 2/2014  | Finley                                |
| 4,589,884 A           | 5/1986           | Gilpatrick         | 2014/0308865 A1 | 10/2014 | Kumar et al.                          |
| 4,680,032 A           | 7/1987           | Arnott             | 2016/0251782 A1 | 9/2016  | Liao et al.                           |
| 4,705,527 A           | 11/1987          | Hussamy            | 2016/0362819 A1 | 12/2016 | Liao et al.                           |
| 5,083,419 A           | 1/1992           | Greifeneder et al. | 2018/0105960 A1 | 4/2018  | Yu et al.                             |
| 5,146,738 A           | 9/1992           | Greifeneder et al. | 2018/0105978 A1 | 4/2018  | Finley                                |
| 5,342,415 A           | 8/1994           | Wasinger           | 2018/0160756 A1 | 6/2018  | Benefiel et al.                       |
| 5,404,626 A           | 4/1995           | Bylund et al.      | 2018/0251939 A1 | 9/2018  | Li et al.                             |
| 5,568,719 A           | 10/1996          | Proctor            | 2019/0284729 A1 | 9/2019  | Chan et al.                           |
| 5,849,040 A           | 12/1998          | Kanehisa           | 2019/0382955 A1 | 12/2019 | Schultz et al.                        |
|                       |                  |                    | 2021/0032805 A1 | 2/2021  | Karaduman et al.                      |

\* cited by examiner

## FIGURE 1

A multilayer article comprising knitted textiles assembled to form the multilayer article that is abrasion resistant, penetration resistant, laceration resistant, and flame resistant

said multilayer article having a

(i) HEAT-TIGHTENED OUTER LAYER comprising a flame resistant, knitted textile made of a first yarn containing modacrylic, cotton and optionally FR rayon, Opan, or aramid fibers; and

(ii) an INNER LAYER comprising a penetration resistant, knitted textile made of a second yarn made from 50-90% HBA/HNA filaments;

wherein the multilayer article is optionally subjected to heat treatment to obtain shrinkage.

## FIGURE 2

Heat-Treated Multilayer Knitted Textile

Flame Resistant Heat-Treated Outer Layer Knitted into a First Layer

attached to

Penetration Resistant Inner Layer Knitted as a Second Layer.

## FIGURE 3

Heat-Treated Multilayer Knitted Textile

Flame Resistant Heat-Treated Outer Layer is

Interlock Knitted with

Penetration Resistant Inner Layer.

## FIGURE 4

Heat-Treated Multilayer Knitted Textile

Flame Resistant Heat-Treated Outer Layer is

plaited with

Penetration Resistant Inner Layer.

## FIGURE 5

ARTICLES MADE FROM  
Heat-Treated Multilayer Knitted Textile

|                   |                |
|-------------------|----------------|
| apparel           | pouches        |
| bags              | pockets        |
| dry bags          | harnesses      |
| inflatable boats  | web-gear       |
| air bags          | hats           |
| footwear          | helmets        |
| insoles for boots | headgear       |
| booties           | shoes          |
| flip flops        | skate shoes    |
| gloves            | insoles        |
| dive gear         | socks          |
| wetsuits          | cuffs          |
| drysuits          | armbands       |
| uniforms          | tents          |
| vests             | armor          |
| flight suits      | carriers       |
| pullovers         | belts          |
| rash guards       | covers         |
| jackets           | furnishings    |
| coveralls         | drapery        |
| shirts            | outdoor fabric |
| trousers          | rope           |
| gear bags         |                |

## FIGURE 6

PROCESS  
for manufacturing

a multilayer knitted textile,  
comprising the step of :

(i) heating a multi-layer knitted textile  
in the presence of one or more dye compounds,  
wherein the multilayer knitted textile comprises  
a fabric outer layer and  
a fabric inner layer,  
wherein the fabric outer layer is knit  
from a first yarn containing a combination of  
modacrylic fibers and cotton fibers,  
wherein the fabric inner layer is knit  
from a second yarn made from 50-90% HBA/HNA filaments,  
wherein the heating shrinks  
the outer layer from about 5 to 25% in length, width, or both.

FIGURE 7

*Image 1: Ring Spun Yarn*

FIGURE 8

*Image 2: Double Knit Interlock Construction*

FIGURE 9



FIGURE 10

| Materials | Density (g/cm <sup>3</sup> ) | Tensile strength (GPa) | Specific strength (km <sup>b</sup> ) | Tensile modulus (GPa) | Specific modulus (km <sup>b</sup> ) |
|-----------|------------------------------|------------------------|--------------------------------------|-----------------------|-------------------------------------|
| HBA/HNA   | 1.4                          | 3.2                    | 229                                  | 75                    | 5300                                |
| Titanium  | 4.5                          | 1.3                    | 39                                   | 110                   | 2300                                |
| Steel     | 7.9                          | 2.0                    | 26                                   | 210                   | 2700                                |
| Aluminum  | 2.8                          | 0.6                    | 22                                   | 70                    | 2600                                |
| E-glass   | 2.6                          | 3.4                    | 130                                  | 72                    | 2800                                |

<sup>a</sup>Specific strength = strength/density (also divided by force of gravity for SI units). Also known as breaking length, the length of fiber that could be held in a vertical direction without breaking

<sup>b</sup>Specific modulus = modulus/density (also divided by force of gravity for SI units). This measure increases with increasing stiffness and decreasing density

FIGURE 11

| Materials | Density (g/cm <sup>3</sup> ) | Tensile strength (GPa) | Tensile modulus (GPa) | Elongation at break (%) | Moisture regain (%) |
|-----------|------------------------------|------------------------|-----------------------|-------------------------|---------------------|
| HBA/HNA   | 1.40                         | 3.4                    | 70                    | 4                       | <0.1                |
| PET       | 1.38                         | 1.1                    | 14                    | 15                      | <0.5                |
| Nylon     | 1.14                         | 1.0                    | 10                    | 28                      | 6-8                 |
| Aramid    | 1.44                         | 3.0                    | 65                    | 4                       | 4-6                 |
| UHMW-PE   | 0.95                         | 3.4                    | 130                   | 4                       | <0.1                |

| Materials | Denier | Relative road |
|-----------|--------|---------------|
| HBA/HNA   | 1500   | 3.4           |
| Aramid    | 1500   | 1.1           |
| UHMW-PE   | 1500   | 1.0           |

|                                        | HBA/HNA | Aramid |
|----------------------------------------|---------|--------|
| LOI                                    | 28      | 30     |
| Melting temperature, °C                | 320     | None   |
| Heat shrinkage at 180 °C for 30 min, % | <0.2    | <0.2   |
| 50 % strength retention temp., °C      | 145     | 400    |
| TGA (20 % weight loss), °C             | >450    | >450   |

FIGURE 12



Plain Weave



Twisted Weave



Dutch Plain Weave



Dutch Twisted Weave

FIGURE 13



FIGURE 14

Flex cycles-to-failure for 400 denier samples and 1.36 kg Load

|          | M Cycles-to-Failure |           |
|----------|---------------------|-----------|
|          | Average             | Range     |
| HBA/HNA  | 18.1                | 16.5-19.8 |
| Aramid A | 1.3                 | 0.7-1.6   |
| Aramid B | 2.2                 | 1.3-3.6   |

FIGURE 15

HBA/HNA HS Tenacity vs. Twists per Inch (TPI)

| TPI | 400 denier tenacity gpd | 1500 denier tenacity gpd |
|-----|-------------------------|--------------------------|
| 0   | 25.6                    | 25.6                     |
| 0.5 | 26.5                    | 26.7                     |
| 1.0 | 27.8                    | 27.6                     |
| 1.5 | 27.8                    | 28.6                     |
| 2.0 | 28.6                    | 27.9                     |
| 2.5 | 28.8                    | 27.6                     |
| 3.0 | 28.1                    | 25.8                     |
| 3.5 | 28.3                    | 24.0                     |
| 4.0 | 28.3                    | 21.8                     |
| 4.5 | 27.8                    | N/A                      |
| 5.0 | 27.8                    | N/A                      |

FIGURE 16



FIGURE 17



FIGURE 18

PROCESS  
for manufacturing

a multilayer knitted textile,  
comprising the step of :

STEP (i) heating a multi-layer knitted textile  
in the presence of one or more dye compounds,  
wherein the multilayer knitted textile comprises  
a fabric outer layer and  
a fabric inner layer,  
wherein the fabric outer layer is knit  
from a first yarn containing a combination of  
modacrylic fibers and cotton fibers,  
wherein the fabric inner layer is knit  
from a second yarn made from 50-90% HBA/HNA filaments,  
wherein the heating shrinks  
the outer layer from about 5 to 25% in length, width, or both.

STEP (ii) assembling the multilayer knitted textile into an article; and

STEP (iii) performing a second heating of the article,  
wherein the second heating further shrinks  
the outer layer from about 2-10% in length, width, or both.

FIGURE 19

## PROCESS FOR MAKING

a double heat-treated protective article having a heat-treated multilayer knitted textile comprising  
a fabric outer layer and  
a fabric inner layer,

Knitting a fabric outer layer  
from a first yarn containing a combination of  
modacrylic fibers and cotton fibers,

Knitting a fabric inner layer  
from a second LCP yarn made from  
50-90% HBA/HNA filaments,

wherein the liquid crystal polymer filaments comprise  
a denier selected from the group consisting of  
200d, 400d, 750d, 1000d, 1420d, 1500d, and 2250d,

wherein the liquid crystal polymer filaments are  
melt spun fibers of a polycondensate of 4-hydroxybenzoic acid (HBA)  
and 6- hydroxynaphthalene-2-carboxylic acid (HNA) monomers (HBA/HNA),

orienting the knit of the fabric inner layer at an  
oblique angle to the knit of the fabric outer  
layer,

attaching the fabric inner layer to the fabric  
outer layer to for a multilayer textile,

heat treating the multilayer textile to obtain shrinkage of 10-15%,

assembling the heat-treated multilayer textile into a protective article and  
heating the protective article to obtain a shrinkage of 4%.

Fig. 20



Fig. 21



## 1

**HEAT TREATED MULTILAYER KNITTED  
TEXTILE OF LIQUID CRYSTAL POLYMER  
FIBERS AND MODIFIED  
POLYACRYLONITRILE FIBERS, AND  
PROCESS FOR MAKING SAME**

**CROSS-REFERENCE TO RELATED  
APPLICATIONS**

Provided by Application Data Sheet per USPTO rules.

**STATEMENT REGARDING FEDERALLY  
SPONSORED R&D**

Provided by Application Data Sheet per with USPTO rules.

**NAMES OF PARTIES TO JOINT RESEARCH  
AGREEMENT**

Provided by Application Data Sheet per with USPTO rules.

**REFERENCE TO SEQUENCE LISTING**

Provided by Application Data Sheet per USPTO rules.

**STATEMENT RE PRIOR DISCLOSURES**

Provided by Application Data Sheet per USPTO rules.

**FIELD OF THE INVENTION**

The invention relates to a multifunctional protective textile for protective garments and accessories made from high strength fibers.

**DESCRIPTION OF THE RELATED ART**

Woven, knitted and nonwoven fabrics are useful in a wide variety of hazardous industrial, medical, military, law enforcement, construction, sports, and home environments where the fabrics may be subjected to sharp objects which can abrade, cut or penetrate the fabric.

For example, U.S. Pat. No. 6,276,255 is a soft body-armor invention touted as being comparatively lightweight, in that a vest made of multilayered sheets or woven fiber antiballistic cloth comprised of ultra high molecular weight polyethylene (UHMWPE) filaments. As with all antiballistic clothing, the antiballistic characteristics are obtained not only from the strength of the materials used, but from the use of multiple layering, both increasing weight and decreasing ease of use.

In another example, U.S. Pat. No. 7,010,811 specifically discloses a soft body-armor product described as lightweight, and claims a material comprising an assembly of woven fabric plies sporting a collective mass per square foot of no more than 1 pound. With such material, a vest for a standard-sized adult would weigh nearly 9 pounds.

Despite their antiballistic qualities, known materials in the soft body armor field have a number of drawbacks. For example, materials such as Kevlar and Dyneema have a tendency to be both substantially heavier and rougher to the touch than synthetic and natural-fiber clothing without anti-ballistic capability. Antiballistic fabrics also tend not to breath, and can cause discomfort and even incapacitate a wearer in environments with high heat and humidity.

## 2

Equally importantly, the qualities that allow antiballistic fabrics to spread and deflect the energy of a ballistic projectile do not provide sufficient protection against non-ballistic forces able to damage the wearer with a puncture or cut, such as nails or knives.

In addition to antiballistic fabrics, there is a need for protective apparel such as gloves that include abrasion-resistant, cut-resistant, thermal resistant, and/or fire-resistant yarn. However, many prior attempts have generated unsatisfactory products, such as being irritating to the skin, being too heavy or inflexible for most applications, having a limited wear life, addressing only one resistance aspect, requiring the use of metal wire or powder fillers, requiring chemical coatings, being difficult to manufacture, or being so uncomfortable to wear or use that it discourages use of the product.

**SUMMARY**

20 The invention relates to a process for manufacturing a heat-treated multifunctional protective textile for protective garments and accessories made from high strength fibers, said garments and accessories are abrasion resistant, improved penetration resistant, laceration resistant, and 25 flame resistant, the textile is made from a flame resistant knitted outer layer made of a first yarn containing modacrylic or aramid fibers; and, a penetration resistant knitted inner layer made of a second yarn made from 50-90% HBA/HNA filaments, as well as methods of manufacturing yarn, methods of manufacturing a textile using the 30 yarn, and apparel made from the yarn.

In order to address the problems in the prior art, the present invention provides herein a preferred embodiment of a process for manufacturing a multilayer knitted textile, comprising the step of (i) heating a multi-layer knitted textile in the presence of one or more dye compounds, wherein the multilayer knitted textile comprises a fabric outer layer and a fabric inner layer, wherein the fabric outer layer is knit from a first yarn containing a combination of 35 modacrylic fibers and cotton fibers, wherein the fabric inner layer is knit from a second yarn made from 50-90% HBA/HNA filaments, wherein the heating shrinks the outer layer from about 5 to 25% in length, width, or both.

In another preferred embodiment, the invention provides 40 wherein the first yarn includes one or more fibers selected from the group consisting of FR rayon fibers, Opan fibers, and aramid fibers.

In another preferred embodiment, the invention provides 45 wherein the fabric outer layer is knit having a wale ranging from 17-27 loops per vertical inch and a course ranging from 18-24 loops per horizontal inch, and wherein after heating, the knit in loops per inch of the fabric outer layer is increased by about 15%.

In another preferred embodiment, the invention provides 50 wherein the fabric inner layer is attached to the fabric outer layer, and the shrinking of the fabric outer layer tightens the knit of the second yarn of the fabric inner layer.

In another preferred embodiment, the invention provides 55 wherein the heating shrinks the outer layer from about 10 to 20% in length, width, or both.

In another preferred embodiment, the invention provides 60 wherein the heating shrinks the outer layer about 15% in length, width, or both.

In another preferred embodiment, the invention provides 65 the process of Step (i) above, comprising the additional steps in order: (ii) assembling the multilayer knitted textile into an article; and (iii) performing a second heating of the article,

wherein the second heating further shrinks the outer layer from about 2-10% in length, width, or both.

In another preferred embodiment, the invention provides wherein the second heating further shrinks the outer layer about 4% in length, width, or both.

In another preferred embodiment, the invention provides wherein the article is selected from the group of products consisting of apparel, bags, dry bags, inflatable boats, air bags, footwear, insoles for boots, booties, flip flops, gloves, dive gear, wetsuits, drysuits, uniforms, vests, flight suits, pullovers, rash guards, jackets, coveralls, shirts, trousers, gear bags, pouches, pockets, harnesses, web-gear, hats, helmets, headgear, shoes, skate shoes, insoles, socks, cuffs, armbands, gloves, tents, armor, carriers, belts, bags, covers, furnishings, drapery, outdoor fabric, and rope.

In another preferred embodiment, the invention provides wherein the liquid crystal polymer filaments comprise a denier selected from the group consisting of 200d, 400d, 750d, 1000d, 1420d, 1500d, and 2250d.

In another preferred embodiment, the invention provides wherein the liquid crystal polymer filaments are melt spun fibers of a polycondensate of 4-hydroxybenzoic acid (HBA) and 6-hydroxynaphthalene-2-carboxylic acid (HNA) monomers (HBA/HNA).

In another preferred embodiment, the invention provides wherein the multilayer textile comprises at least one additional fabric layer.

In another preferred embodiment, the invention provides wherein the fabric inner layer is attached to the fabric outer layer using a knitting technique, is sewn, is interlock knitted to, or is plaited with the fabric outer layer as an overbraid.

In another preferred embodiment, the invention provides wherein the knit of the fabric inner layer is oriented at an oblique angle to the knit of the fabric outer layer.

In another preferred embodiment, the invention provides wherein the knit of the fabric inner layer is oriented at an orthogonal angle to the knit of the fabric outer layer.

In another preferred embodiment, the invention provides wherein the one or dyes are disperse dyes selected from the group consisting of: Nitro Dyes, Amino Ketone dyes, Anthraquinonoid dyes, Mono azo dyes, Di-azo dyes, and mixtures thereof.

In another preferred embodiment, the invention provides wherein the disperse dyes are applied using a method selected from the group consisting of: Normal dyeing method at a Dyeing temperature 80-100° C., a Normal Method of dyeing with carriers at a Dyeing temperature 80-100° C., a High temperature dyeing method at a Dyeing temperature 105-140° C., a Thermasol dyeing method at a Dyeing temperature 180-220° C., a Semi continuous Pad roll dyeing method, and a Continuous Pad steam method.

In another preferred embodiment, the invention provides a double heat-treated protective article, having a heat-treated multilayer knitted textile, the heat-treated multilayer knitted textile comprising a fabric outer layer and a fabric inner layer, wherein the fabric outer layer is knit from a first yarn containing a combination of modacrylic fibers and cotton fibers, wherein the fabric inner layer is knit from a second yarn made from 50-90% HBA/HNA filaments, wherein the liquid crystal polymer filaments comprise a denier selected from the group consisting of 200d, 400d, 750d, 1000d, 1420d, 1500d, and 2250d, wherein the liquid crystal polymer filaments are melt spun fibers of a polycondensate of 4-hydroxybenzoic acid (HBA) and 6-hydroxynaphthalene-2-carboxylic acid (HNA) monomers (HBA/HNA), wherein the knit of the fabric inner layer is oriented at an oblique angle to the knit of the fabric outer layer, wherein the fabric

outer layer is attached to the fabric inner layer, wherein the heat-treated multilayer knitted textile is pre-shrunk about 10-15%, and wherein the protective article is secondarily heat-shrunk an additional 4%.

In another preferred embodiment, the invention provides wherein the article is selected from the group of products consisting of apparel, bags, dry bags, inflatable boats, air bags, footwear, insoles for boots, booties, flip flops, gloves, dive gear, wetsuits, drysuits, uniforms, vests, flight suits, pullovers, rash guards, jackets, coveralls, shirts, trousers, gear bags, pouches, pockets, harnesses, web-gear, hats, helmets, headgear, shoes, skate shoes, insoles, socks, cuffs, armbands, gloves, tents, armor, carriers, belts, bags, covers, furnishings, drapery, outdoor fabric, and rope.

#### BRIEF DESCRIPTION OF THE DRAWINGS

FIG. 1 is a text graphic showing one preferred embodiment of the main components of the present invention.

FIG. 2 is a text graphic and shows one option for attaching the first layer to the second layer.

FIG. 3 is a text graphic and shows a second option for attaching the first layer to the second layer.

FIG. 4 is a text graphic and shows a third option for attaching the first layer to the second layer.

FIG. 5 is a text graphic list of the inventive articles that can be made from the textile invention described herein.

FIG. 6 is a text graphic and represents process for manufacturing the multilayer knitted textile of the present invention.

FIG. 7 is a graphic representation of a three-layer ring spun yarn.

FIG. 8 is a graphic representation of a double knit interlock textile construction.

FIG. 9 is a drawing showing the orientation of fibers in a liquid crystal polymer compared to a polyester fiber.

FIG. 10 is a table comparing the strength of HBA/HNA against other materials.

FIG. 11 is a table comparing the strength of HBA/HNA against other polymer fibers.

FIG. 12 is a drawing of four different types of weave patterns.

FIG. 13 is a photomicrograph of 12 different types of weave patterns.

FIG. 14 is a table showing the number of cycles in a flex test before a fiber fails, and compares HBA/HNA against aramid fibers.

FIG. 15 is a table showing the tenacity of HBA/HNA as it relates to the number of twists per inch in a yarn construction.

FIG. 16 is a table showing the breaking load of HBA/HNA fibers comparing an S-twist versus a 3-ply Z twist.

FIG. 17 is a table showing the difference in tenacity under UV stress between a HBA/HNA filament yarn with and without a polyester over-braid/sheath.

FIG. 18 is a flowchart showing certain method steps according to the present invention.

FIG. 19 is a illustration of the feature of a double heat-treated protective article, having a heat-treated multilayer knitted textile, according to the present invention.

FIG. 20 is a non-limiting illustration of the two layer fabric, with a first layer having, e.g. cotton and modacrylic, and the second layer having a liquid crystal polymer knit fabric.

FIG. 21 is a non-limiting illustration of the heating and dyeing process of the two layer fabric, with a first layer having, e.g. cotton and modacrylic, having a wider knit,

smaller number of loops per inch, before heating, and having a tighter, narrower knit, a greater number of loops per inch, after the heating. Since LCP textiles are difficult to dye, the addition of the first layer provides a (two-layer) dyed textile having the strength, puncture-resistance, cut-resistance, chemical resistance, and light weight characteristics of the underlying LCP textile while having the colorability, soft-feel, and fire-resistance of the modacrylicblend. Additionally, the heat shrinkage, and increase in loop density, of the first layer, is joined by a parallel increase in loop density of the second layer since the two layer are attached, e.g. quilter, together. The shrinkage of the first layer causing an increased tightness of knit in the second layer adds a significant degree of strength and enhanced performance characteristics to the second LCP layer.

#### DETAILED DESCRIPTION OF THE INVENTION

The embodiments herein and the various features and advantageous details thereof are explained more fully with reference to the non-limiting embodiments that are illustrated in the accompanying drawings and detailed in the following description. Descriptions of well-known components and processing techniques are omitted so as to not unnecessarily obscure the embodiments herein. The examples used herein are intended merely to facilitate an understanding of ways in which the embodiments herein may be practiced and to further enable those of skill in the art to practice the embodiments herein. Accordingly, the examples should not be construed as limiting the scope of the embodiments herein.

Rather, these embodiments are provided so that this disclosure will be thorough and complete, and will fully convey the scope of the invention to those skilled in the art. Like numbers refer to like elements throughout. As used herein the term “and/or” includes any and all combinations of one or more of the associated listed items.

The terminology used herein is for the purpose of describing particular embodiments only and is not intended to limit the full scope of the invention. As used herein, the singular forms “a”, “an” and “the” are intended to include the plural forms as well, unless the context clearly indicates otherwise. It will be further understood that the terms “comprises” and/or “comprising,” when used in this specification, specify the presence of stated features, integers, steps, operations, elements, and/or components, but do not preclude the presence or addition of one or more other features, integers, steps, operations, elements, components, and/or groups thereof.

Unless otherwise defined, all terms (including technical and scientific terms) used herein have the same meaning as commonly understood by one of ordinary skill in the art to which this invention belongs. It will be further understood that terms, such as those defined in commonly used dictionaries, should be interpreted as having a meaning that is consistent with their meaning in the context of the relevant art and will not be interpreted in an idealized or overly formal sense unless expressly so defined herein.

#### Dye

A dye is an organic colored compound for adding color to a textile and which chemically binds to the fibers of the textile substrate.

Dyestuff consists of chromophores and auxochromes. Chromophores give the dye molecule its particular color, while the auxochromes intensify the hue of the dye molecule's color, increases solubility of the dye molecule, and

improves the color fastness of the dyed or printed fabric. Chromophores groups include azo, quinonoid, nitro and nitroso groups whereas auxochromes include acidic moieties, such as carboxylic acid and sulphonate acid groups, and basic moieties such as amino groups and hydroxyl groups.

#### Substantivity

This dye characteristic is the tendency of a dye to move out of a solution and into fibers. The substantivity of dyes depend upon Molecular structure (shape), Size of molecule dye, and Dye bath conditions. The degree of substantivity reflects the amount of dye that is applied, or exhausted onto, to the fiber under neutral conditions.

#### Affinity

In dyeing, affinity refers to the preferential attraction of the dye for the fiber rather than for the solution of the dye bath. It is quantitative unit for expressing substantivity. Affinity is expressed in term of energy. Generally, more substantive dyes have low affinity characteristic.

#### Exhaustion

The process of transfer of dyestuff from the dye bath on to the fiber or material is known as exhaustion. The ratio between the amount of dye taken up by the substrate and the amount of dye originally available. Exhaustion is overall broad term and can be further categorized into two phases. Primary exhaustion is the phase where dye moves toward the substrate from the solution under neutral conditions in the presence of electrolyte. It is also known as substantive phase. The term secondary is typical movement of dye molecule after addition of dye molecules after addition of suitable alkali for the completion of the dye fiber bonding.

The exhaustion of dyestuff depends upon: the Concentration of dye, Concentration of salt, Temperature, Agitation, and the liquor ratio.

#### Adsorption

Dyes molecules from solution are taken up by certain textile substrates which have porous surface i.e. cotton is characterized by adsorption. Distribution of the dye stuff on to the surface of the fiber is known as adsorption. Adsorption depends upon: the Concentration, Temperature, Dye type, Pressure, and Surface area.

#### Absorption

The term absorption refers to the distribution of the dye-stuff containing liquor as applied to the whole surface of fiber. Certain factors affect the rate of absorption, including: Time in proximity to dye, Temperature, Alkali treatment, Electrolytes, Dyeing Auxiliaries, and the Liquor ratio.

#### Diffusion

The term diffusion refers to the process by which the dye moves from the surface of the fiber into the matrix, pores, and/or interstices of the macromolecular and molecular structure of the fiber itself. The diffusion rate of given dyestuff is heavily influenced by temperature. The higher the temperature, the greater the degree and rate of diffusion. The diffusion rate can also depend on the crystallinity of the fabric structure.

#### Zeta Potential

The term Zeta potential refers to the difference in electrical potential across the interface (a diffuse double layer) of a solid surface contact with a liquid.

#### Fixation

The term fixation refers to the formation of the “final” bond between the dye and the fiber by mechanisms including ionic bonding and hydrophobic forces. Dispersion dyes and vat dyes are fixed in the fiber largely by physical entrapment of insoluble dye within the fibre. The chemical

bond that causes final fixation is not necessarily the same type of chemical bond that occurs when a dye is first applied to a fiber.

#### Reactivity

The term reactivity refers to the rate at which a dye reacts with fiber. High reactivity dyes react rapidly at relatively low temperature, whereas low reactivity dyes generally require relatively high temperature for dye fixation.

#### Types of Dyeing

There are multiple types of dyeing methods. Garment dyeing Dye is applied to finished products such as apparel and garments. Stock dyeing is used to dye fibers. In this process, the staple fibers are packed into a vessel and then dye liquid is forced through them. Woolens are usually stock dyed. Yarn dyeing refers to when dyeing is done after the fiber has been spun into yarn. In this method, the dyestuff penetrates the fibers to the core of the yarn. There are many forms of yarn dyeing-Skein (Hank) Dyeing, Package Dyeing, Warp-beam Dyeing, and Space Dyeing.

#### Ultrasonic Assisted Dyeing

The use of ultrasound in the dyeing of textile refers to when ultrasound waves are applied to the liquid dye system in order to generate the phenomenon of cavitations. U/S/ generated cavitations liberate entrapped gases from liquid or porous material like textiles, dyebath etc., and affect the dye's ability to disperse and diffuse

#### Microwave Dyeing

Microwave dyeing takes into account only the dielectric and the thermal properties. The dielectric property refers to the intrinsic electrical properties that affects the dyeing by polar rotation of the dye & influences the microwave field upon the dipoles. The aqueous solution of dye has two components which are polar, dye molecules and water molecules. In a microwave field oscillating at 2.45 GHz, the vibrational energy in the water molecules and the dye molecules generate heat and results in collision of dye molecules with the molecules of the fiber. Using a mordant during this process can assist penetration of the dye and increase the depth of dye penetration into the fabric.

#### Electrochemical Dyeing

Some dyes are insoluble in water, and using them makes it necessary to convert them into water-soluble form using suitable reducing agent and alkali.

#### Supercritical Carbon Dioxide (CO<sub>2</sub>) Dyeing

Converting carbon dioxide into a super critical fluid in order to replace water as a dye solvent can provide high diffusion rates and low viscosities that allow the dye to better penetrate into the fiber. Using supercritical CO<sub>2</sub> also reduces the pressure at the end of the process, thereby allowing unused dye and CO<sub>2</sub> to be recycled.

#### Dyeing Aramids and LCPs

Advanced fibers have a rigid molecular structure that requires special conditions for dyeing. Certain cationic (basic) dyes may include Yellow 13, 21, 28 and 29, Red 29, Blue 3, 41, and 54, and Black mixture. Carriers typically include glycol (aryl)ether, acetophenone, n-methylformanilide, benzyl alcohol, phthalimide, and mixtures thereof. Concentrations range from 30-100 g/L. Sodium nitrate is also used in the dyebath, along with acetic acid, lubricants, chelators, and anti-foaming agents. Dyeing temperatures may include a first reaction (Phase 1) at 150 degrees F. with the dyestuff, carriers, pH conditioners and sodium nitrate. Phase 1 is then followed by a temperature increase (Phase 2) to 265 degrees F. for a specified period. In Phase 3, the temperature is lowered again, e.g. to 175 degrees F. for draining and scouring.

#### Dyeing Modacrylic

Modacrylic requires basic dyes (cationic), that links with an anionic dye site on the fiber. Modacrylic also has a limited dyeing temperature of between 212-217 degrees F. Exceeding this temperature will generate shrinkage. Modacrylic also has a glass transition temperature where the fiber structure opens and allows better dye strike at 194-203 degrees F. In Phase 1, the temperature is held at 140 degrees F. for dyebath and dyestuff. In Phase 2, the temperature is raised to between 212-225 degrees F. and held for up to 30-120 minutes. In Phase 3, the temperature is lowered to 100-140 for washing and softening. Typical dyebath includes acetic acid pH 3.5-5.0, sodium sulfate, a retarder/leveler, a nonionic lubricant, and a non-silicone foam control agent.

#### Dyeing FR Rayon

Rayon can be direct or Vat dyed. FR Rayon may also require an exhaust procedure having a low temperature 90 deg. F dyebath and electrolyte Phase 1 for about 60 minutes, followed by a 140 deg. F alkali Phase 2 for about 90 minutes, followed by discrete washing, soaping, and fixative phases over the remaining 250 minutes. FR Rayon direct dye may include a 45 minute dyebath and dyestuff Phase 1 at 110 deg. F, followed by a 120 min. electrolyte Phase 2 at 200 deg. F, followed by a low temperature cold rinse, electrolyte rinse and fixative Phases at 110-130 deg. F.

#### Dyeing Vectran/HBA-HNA Filaments

These engineered fibers are known to be difficult to dye. In fact, these fibers are specifically designed to resist chemical and temperature attack, which makes dyeing them next to impossible. However, in a multilayer fabric, using other fibers, dyeing can be accomplished. Further, using the inventive process herein, the shrinkage of the other fibers can, when mated or attached to the engineered filament knits, be used to tighten down the knit structure and create a stronger, more resistant fabric.

#### Knit Tightening

Knit structure is known to create wales—vertical, stacked loops—and course—horizontal, adjacent interlocked loops. Because of this structure, a knit fabric will shrink or tighten more in the vertical direction, and slightly less so in the horizontal direction. However, such tightening of the loops, using heat effect of the fibers, will reduce the space in the gaps, thus leading to a tighter loop structure. For example if a knit textile is knit having between 17-27 loops per inch. After heat effect shrinkage, the loop rate will increase by up to 15% or more, e.g. 19.5-31 loops per inch.

Referring now to FIG. 1, FIG. 1 is a text graphic showing one preferred embodiment of the main components of the present invention, namely a multilayer knitted textile, comprising: (i) at least one flame resistant knitted outer layer made of a first yarn containing modacrylic or aramid fibers; and, (ii) at least one penetration resistant knitted inner layer made of a second yarn made from 50-90% HBA/HNA filaments.

FIG. 2 is a text graphic and shows one option for attaching the first layer to the second layer in a multilayer knitted textile, wherein the at least one flame resistant knitted outer layer uses a knitting technique, or is sewn, to the at least one penetration resistant knitted layer.

FIG. 3 is a text graphic and shows a second option for attaching the first layer to the second layer in a multilayer knitted textile, wherein the at least one flame resistant knitted outer layer is interlock knitted to the at least one penetration resistant knitted layer.

FIG. 4 is a text graphic and shows a third option for attaching the first layer to the second layer in a multilayer

knitted textile, wherein the at least one flame resistant knitted outer layer is plaited with the at least one penetration resistant knitted layer as an overbraid.

FIG. 5 is a text graphic list of the inventive articles that can be made from the textile invention described herein. Specifically, the article may be apparel, bags, dry bags, inflatable boats, air bags, footwear, insoles for boots, booties, flip flops, gloves, dive gear, wetsuits, drysuits, uniforms, vests, flight suits, pullovers, rash guards, jackets, coveralls, shirts, trousers, gear bags, pouches, pockets, harnesses, web-gear, hats, helmets, headgear, shoes, skate shoes, insoles, socks, cuffs, armbands, gloves, tents, armor carriers, belts, bags, covers, furnishings, drapery, outdoor fabric, and rope.

FIG. 6 is a text graphic and represents five (5) broad process steps for manufacturing the multilayer knitted textile of the present invention. The process for manufacturing a multilayer knitted textile is illustrated in the steps: (i) providing a first yarn containing modacrylic or aramid fibers; (ii) knitting the first yarn into a fabric outer layer; (iii) providing a second yarn made from 50-90% HBA/HNA filaments; (iv) knitting the second yarn into a fabric inner layer; and (v) assembling where the knitting technique creates the fabric outer layer and the fabric inner layer into a multilayer knitted textile.

Referring now to FIG. 7, there is shown a drawing of a ring-spun yarn. In ring-spun yarns, twisting takes place from the outside inwards. At the periphery (the outer sheath A, owing to the greater degree of winding, the fibers have a lesser inclination, ( $\gamma$ =angle between the fibers and the axis of the yarn) than in the interior of the yarn (the core B). Since the fibers become steadily less tightly wound towards the core, ring-spun yarn may be said to have sheath-twist. Under loading, the outer layers will tend to take the radial forces and the inner layers will tend to take the axial forces. However, by increasing pressure inwards, the radial forces reinforce axial resistance to sliding apart of the fibers. Accordingly, fully twisted yarns with sheath-twist have high tensile strength but are not so resistant to abrasion.

Denier: is a unit of measure for the linear mass density of fibers. It is defined as the mass in grams per 9000 meters, or more commonly, weight in milligrams of a 9 meters strand. 1 denier=0.11 mg/m. The denier is based on a natural reference—i.e., a single strand of silk is approximately one denier. A 9000-meter strand of silk weighs about one gram. The term denier comes from the French denier, a coin of small value. Applied to yarn, a denier was held to be equal in weight to  $\frac{1}{24}$  of an ounce. The term microdenier is used to describe filaments that weigh less than one gram per 9000 meters.

One can distinguish between filament and total measurements in deniers. Both are defined as above but the first only relates to a single filament of fiber—commonly known as denier per filament (DPF)—whereas the second relates to a yarn, a spun agglomeration of filaments. Broader terms such as ‘fine’ may be applied because either the overall yarn is fine or because fibers within this yarn are thin. 75 denier yarn would be considered fine even if it only contains a few fibers, such as thirty 2-denier fibers, but a heavier yarn such as 150 denier is only considered fine if its constituent fibers are individually as thin as 1 denier.

The following relationship applies to straight, uniform filaments:

DPF=total denier/quantity of uniform filaments

The denier system of measurement is used on two- and single-filament fibers. Some common calculations are as follows:

1 denier=1 gram per 9 000 meters=0.111 milligrams per meter

In practice, measuring 9000 meters is both time-consuming and unrealistic; generally a sample of 900 meters is weighed and the result multiplied by 10 to obtain the denier weight.

10 A fiber is generally considered a microfiber if it is one denier or less.

A one-denier polyester fiber has a diameter of about ten micrometers.

15 One can calculate the diameter of a filament yarn using denier with the following formula (where density is in grams per cubic centimeter and the diameter is in mm):

$$\text{Diameter} = \sqrt{\frac{\text{Denier}}{9000 \cdot \text{density} \cdot 0.7855}}$$

#### Fiber Strength (Tenacity):

Another linear mass density unit is called tex. The Tensile Strength expressed as force per unit liner density is called tenacity. (units of cN/tex). This is normally expressed as gram force per tex (gf/tex)=dtex (deci)=grams/10,000 m. Note: The higher the value, the better the strength of the 25 yarn. Units g.dTex refers to grams per deci-tex (0.1 of tex)(tex=1 mg/m, weight to length ratio).

#### Yarn

The invention begins with a novel yarn construction, providing high-level durability and trauma resistance, while 35 still feeling and behaving as standard apparel fabric when woven appropriately. The term yarn generally refers without limitation to a long continuous length of interlocked fibers suitable for use in the production of textiles, sewing, knitting, weaving, rope making, and the like.

#### 40 Composites

A composite is a solid material, made out of two or more constituent, different and distinct substances that retain their physical characteristics, while contributing desirable properties to the whole. Composite materials generally include 45 three functions. A matrix function feature that surrounds, supports and maintains position of a reinforcement. A reinforcement function feature that provides one or more special physical characteristics, e.g. mechanical or electrical. And a core function feature used in-between the layers of fiber 50 reinforced matrix forming a type of sandwich structure. When matrix and reinforcement are combined in a laminate to form a new material, this can result in a synergistic characteristic or feature.

Some of the benefits of composite materials include 55 higher mechanical properties like strength and stiffness, lighter weight, higher performance, energy savings, durability, fatigue resistance and longer service life, impact resistance, dimensional stability, anisotropic properties, chemical properties, corrosion resistance, fire retardance, 60 high temperature service, environment outdoor service, low maintenance requirements, low thermal conductivity, low or custom thermal expansion, tailored energy conductivity, (e.g. can be used to amplify or damp vibration), tailored transparency to radio frequency (reflection or dumping 65 properties), tailored electric properties (insulation or conduction capability), tailored electromagnetic transparency, tailored properties for both telecommunication and stealth

## 11

technologies, flexible, tailor design, part consolidation and freedom of shape, and so forth.

## Hybrid Composite Constructions

Included within the scope of the invention are yarn constructions and tow constructions.

Yarn is a twisted bundle of filaments, which may be continuous or non-continuous. Tow is an untwisted bundle of continuous filaments.

Referring now to FIG. 8, there is shown an example of a double knit interlock construction. Textile is constructed using a double-knit modified interlock construction. Double knitting is a form in which two fabrics are knitted simultaneously on one pair of needles. The fabrics may be inseparable, as in interlock knitted fabrics.

Referring now to FIG. 9, comparing the orientation of polyester fibers versus the order orientation of HBA/HNA fibers, HBA/HNA is capable of forming regions of highly ordered structure while in the liquid phase. However, the degree of order is somewhat less than that of a regular solid crystal. Typically LCPs have a high mechanical strength at high temperatures, extreme chemical resistance, inherent flame retardancy, and good weatherability. Liquid-crystal polymers come in a variety of forms from sinterable high temperature to injection moldable compounds. LCP can be welded, though the lines created by welding are a weak point in the resulting product. LCP has a high Z-axis coefficient of thermal expansion.

In comparison, conventional polyethylene terephthalate (PET) has flexible molecular chains, and the as-spun fiber from PET has a low molecular orientation giving it a low strength and limiting its industrial use.

In comparison to aramids like Kevlar, Kevlar must be solvent spun due to its lyotropic nature. In comparison to ultrahigh molecular weight polyethylene (UHMWPE), UHMW-PE must be gel spun in order to control the density of chain entanglements.

LCPs are exceptionally inert. They resist stress cracking in the presence of most chemicals at elevated temperatures, including aromatic or halogenated hydrocarbons, strong acids, bases, ketones, and other aggressive industrial substances. Hydrolytic stability in boiling water is excellent. Environments that deteriorate the polymers are high-temperature steam, concentrated sulfuric acid, and boiling caustic materials.

Melt Spun HBA/HNA, aka ms-HBA/HNA or MS-HBA/HNA, is a multifilament yarn spun from liquid crystal polymer (LCP). HBA/HNA is the only melt spun yarn commercially available. HBA/HNA is an aromatic polyester spun from LCP in melt extrusion. Chemically, HBA/HNA is produced from polycondensation of 4-hydroxybenzoic acid and 6-hydroxynaphthalene-2-carboxylic acid.

[4-hydroxy-benzoic acid] and  
[6-hydroxy-naphthalene-2-carboxylic acid]



## 12

Liquid-crystal polymers (LCPs) are a class of aromatic polyester polymers. They are extremely unreactive and inert, and highly resistant to fire.

HBA/HNA is melt-processed on conventional equipment at high speeds with excellent replication of mold details and the high ease of forming of LCPs is an important competitive advantage against other plastics, as it offsets high raw material cost.

10 HBA/HNA is a thermotropic liquid crystalline copolymer composed of 4-hydroxybenzoic acid (HBA) and 2-hydroxy-6-naphthoic acid (HNA) monomers in specific molar ratios of HBA/HNA. In one preferred embodiment, the molar ratio ranges from 50-90% HBA to 10-50% HNA. In another preferred embodiment, the molar ratio ranges from 60-85% HBA to 15-40% HNA. In another preferred embodiment, the molar ratio ranges from 65-75% HBA to 25-35% HNA. In another preferred embodiment, the molar ratio equals about 3 moles HBA to 1 mole HNA. In another preferred embodiment, the molar mass ratio equals HBA to HNA in a ratio of about 73 to 27.

15 168. Referring now to FIG. 10, comparing HBA/HNA Strength vs. Other Materials, HBA/HNA has the lowest density (g/cm<sup>3</sup>) with the highest specific strength (km<sup>2</sup>) and specific modulus (km<sup>3</sup>).

20 Referring now to FIG. 11, comparing HBA/HNA Strength vs. Other Fibers, HBA/HNA matches aramid fiber and UHMW-PE fibers for density, tensile strength, low elongation at break, and low moisture regain percentage.

25 Referring also to FIG. 11, comparing HBA/HNA Cut Resistance, HBA/HNA has nearly three times the score compared to aramid and UHMW-PE fibers at similar deniers.

30 Referring again to FIG. 11, comparing HBA/HNA Thermal Resistance versus aramid fibers, HBA/HNA shows excellent thermal resistance compared to aramids.

35 40 Referring now to FIG. 14, FIG. 14 is a table showing the number of cycles in a flex test before a fiber fails, and compares HBA/HNA against aramid fibers. FIG. 14 shows how HBA/HNA ranges from 9-14 times the number of cycles that aramid does before breaking.

45 Referring now to FIG. 15, FIG. 15 is a table showing the tenacity of HBA/HNA as it relates to the number of twists per inch in a yarn construction. FIG. 15 shows how the ideal number of twists per inch is around 2.5, but also that tenacity is excellent across a range of TPI.

50 55 Referring now to FIG. 16, FIG. 16 is a table showing the breaking load of HBA/HNA fibers comparing an S-twist versus a 3-ply Z twist. FIG. 10, shows that HBA/HNA can be used successfully in complex or hybrid yarns, and that HBA/HNA increases in strength when the complexity of the twisted composite fiber is increased.

60 Referring now to FIG. 17, FIG. 17 is a table showing the difference in tenacity under UV stress between a HBA/HNA filament yarn with and without a polyester over-braid/sheath. FIG. 17 shows that using a UV sheath or overbraid is an effective way to manage the single weak aspect of HBA/HNA fibers, UV exposure.

65 65 Modified polyacrylonitrile (M-PAN) is a co-polymer having from 35% to 85% acrylonitrile that has been modified by halogen containing co-monomers including polyvinyl chloride known as Dynel® and/or with vinylidene chloride known as Verel®.



Polyacrylonitrile is a polymer of acrylonitrile monomers.



#### Polyacrylonitrile

M-PAN is a synthetic copolymer. M-PAN polymer fibers, yarns, and fabrics are soft, strong, resilient, and dimensionally stable. They can be easily dyed, show good press and shape retention, and are quick to dry. They have outstanding resistance to chemicals and solvents, are not attacked by moths or mildew, and are nonallergenic. Among their uses are in apparel linings, furlike outerwear, paint-roller covers, scatter rugs, carpets, and work clothing and as hair in wigs.

M-PAN fibers are modified acrylic fibers made from acrylonitriles, but larger amounts of other polymers are added to make the copolymers. The M-PAN fibers are produced by polymerizing the components, dissolving the copolymer in acetone, pumping the solution into the column of warm air (dry-spun), and stretching while hot.

M-PAN fibers are creamy or white and are produced in tow and staple form. If looked at in cross section views they have an irregular shape. M-PAN fibers are also produced in many different lengths, crimp levels, deniers and they can have various shrinkage potentials.

The Federal Trade Commission defines M-PAN fibers as manufactured fibers in which the fiber-forming substance is any long-chain synthetic polymer composed of less than 85%, but at least 35% weight acrylonitrile units except when the polymer qualifies as rubber.

A M-PAN has properties that are similar to an acrylic. However, M-PANs are flame retardant and do not combust. The fibers are difficult to ignite and will self-extinguish. In addition to a M-PAN's flame retardant properties it has a relatively high durability that is comparable to wool. M-PAN fibers have a moderate resistance to abrasion and a very low tenacity. One of the most interesting properties of M-PAN fabrics is the arc flash protection, where it has very good values. M-PANs are poor conductors of heat. The fabrics are soft, warm and resilient but are prone to pilling and matting. M-PANs display high performance when it comes to appearance retention. The fibers are quite resilient and will not wrinkle. They also have great dimensional stability and high elastic recovery, which gives them the ability to hold their shape.

M-PANs are used primarily in applications where environmental resistance or flame retardancy is necessary or required. M-PANs have the ability to combine flame retardancy with a relatively low density, meaning protective gear is not uncomfortably heavy (i.e. shirts and trousers worn by

electrical linemen). The combination of flame retardancy and low density is also useful in furnishings, draperies, and outdoor fabrics.

#### Example 1—Sheathed Ring Spun Yarn

In one preferred embodiment, the invention provides a co-extruded filament hybrid composite sheathed with a second filament. In this example, 400d (denier) HBA/HNA (V1) and M-PAN (M) are melt co-extruded in a 90-10 ratio (V1:M) through fine diameter capillaries resulting in a first component filament (F1), and the first strand (F1) is then ring-spun into a multi-layer ring-spun yarn (RS), the multi-layer ring spun yarn is then sheathed with a HBA/HNA (V2) filament in a 10:90 ratio (RS:V2), to form a sheathed ring spun yarn (SRS).

#### Example 2—Double Twisted Yarn

In one preferred embodiment, the invention provides a hybrid composite double twisted yarn. In this example, a 400d (denier) HBA/HNA (V1) filament and M-PAN (M) filament are twisted in a 90-10 ratio (V1:M) resulting in a first component twisted filament (TF1), and the first twisted filament (TF1) is then ring-spun into a multi-layer ring-spun yarn (RS), the multi-layer ring spun yarn is then sheathed with a HBA/HNA (V2) filament in a 10:90 ratio (RS:V2), to form a sheathed ring spun yarn (SRS).

#### Example 3—Filament Core Double Twisted Yarn

In one preferred embodiment, the invention provides a hybrid composite filament core double twisted yarn. In this example, a 400d (denier) HBA/HNA (V1) filament and M-PAN (M) filament are twisted in a 90-10 ratio (V1:M) resulting in a first component twisted filament (TF1), and the first twisted filament (TF1) is then ring-spun into a multi-layer ring-spun yarn (RS), the multi-layer ring spun yarn is then used to sheath a HBA/HNA (V2) core filament, in a 10:90 ratio (RS:V2), to form a filament core ring-spun sheathed yarn (FCRSS).

#### Example 4—Sheathed Ring-Spun Tow (Non-Yarn)

In one preferred embodiment, the invention provides a sheathed ring-spun tow hybrid composite. In this example, 400d (denier) HBA/HNA filament (V1) and M-PAN (M) are bundled as an untwisted tow in a 90-10 ratio (V1:M) resulting in a first component bundle filament (B1), and the first component bundle filament (B1) is then ring-spun into a multi-layer ring-spun yarn (RS), the multi-layer ring spun yarn is then sheathed with a HBA/HNA (V2) filament in a 10:90 ratio (RS:V2), to form a sheathed ring spun yarn (SRS).

#### Example 5—Double Co-Extruded Tow (Non-Yarn)

In one preferred embodiment, the invention provides a co-extruded filament hybrid composite. In this example, 400d (denier) HBA/HNA (V1) and M-PAN (M) are melt co-extruded in a 90-10 ratio (V1:M) through fine diameter capillaries resulting in a first component strand (S1), and the first strand (S1) is then melt co-extruded with HBA/HNA (V2) in a 10:90 ratio (S1:V2), to form a double co-extruded hybrid composite filament (S2), which is then used to make a yarn and textile.

## 15

## Example—Double Knit Interlock Textile

Referring again to FIG. 8, there is shown an example of a double knit interlock construction. Textile is constructed using a double-knit modified interlock construction. Double knitting is a form in which two fabrics are knitted simultaneously on one pair of needles. The fabrics may be inseparable, as in interlock knitted fabrics, or they can simply be two unconnected textiles. A double knit interlock will create a fabric that can be rib-like in appearance on one or both sides.

Knitting creates a V-shape on one side of a fabric, with loops (pearls) on the back side. A double-knit will have two fabrics back-to-back with their inner loops adjacent one another and the outer V-pattern facing in opposite directions. These fabrics show good dimensional stability and are easy to cut and sew. They do not require any seam finishes, as the fabric does not unravel. They are firm, heavier, low stretch and more resilient, making them an ideal candidate when designing durable textiles. Interlocking is the process of taking connecting the back side loops together by alternatively jumping the yarn from one fabric to the other and back.

## Optional Resins

In a preferred embodiment, the composite may be constructed using a combination of fiber reinforcement and a resin matrix. The resin system holds everything together, and transfers mechanical loads through the fibers to the rest of the structure. In addition to binding the composite structure together, it protects from impact, abrasion, corrosion, other environmental factors and rough handling. Resin systems come in a variety of chemical families, each designed and designated to serve industries providing certain advantages like economic, structural performance, resistance to various factors, legislation compliance, etc. Resins of the thermoset family are described below, and include polyester (orthophthalic and isophthalic), vinyl ester, epoxy, and phenolic.

**Polyester resins**—Unsaturated polyester resins are the simple, economical resins that are easy to prepare and show good performance. They are manufactured by the condensation polymerization of various diols (alcohols) and dibasic acids (e.g. maleic anhydride or fumaric acid) to give esters, a very viscous liquid that is then dissolved in styrene, a reactive monomer. Styrene lowers the viscosity to a level suitable for impregnation or lamination.

**Orthophthalic resins**—also referred to as ortho or General Purpose Polyester (GP) was the original polyester developed. It has a low cost and is used in applications where high mechanical properties, corrosion resistance, and thermal stability are not required.

**Isophthalic resin**—is an improved polyester. It has a slightly higher cost, improved strength, thermal stability (55° C.) and mild resistance to corrosion conditions. It has improved resistance to water permeation and improved chemical resistance.

**Vinyl ester**—another improved polyester, is bisphenol chlorinated, or a combination of polyester and epoxy. Its curing, handling and processing characteristics are those of polyester, and it exhibits higher test results in corrosion temperature resistance and strength. Modifications of the molecule can provide tailored properties.

**Phenolic resin**—is a reaction of phenol and formaldehyde. It can be cured via heat and pressure, without the use of catalysts or curing agents. Cured phenolic resins are fire resistant without the use of mineral fillers or fire retardant

## 16

additives. Phenolic composites have excellent high-temperature properties. Phenolics are also unique in their chemical resistance.

**Epoxy resins**—are a broad family of materials. The most common ones are prepared from the reaction of bis-phenol A and epichlorohydrin and contain a reactive functional group in their molecular structure. Epoxy resin systems show extremely high three dimensional crosslink density which results to the best mechanical performance characteristics of all the resins. The most demanding strength/weight applications use epoxy almost exclusively. It has excellent strength and hardness, very good chemical heat and electrical resistance.

**Gel coats**—are prepared from a base resin and additives. The base resin can be polyester, vinyl ester, phenolic or epoxy. Additives are thixotropic agents, fillers, pigments and other. The gel coat, as the name implies, has a gel texture. This makes the gel coat capable to “stay” on vertical surfaces of molds without draping. It is placed first in the mold, so it becomes the outer surface of the construction.

## Textiles, Fabric

The instant invention relates to multifunctional protective textiles (syn. fabrics) for protective garments and accessories made from high strength fibers and materials, as well as methods for making such multifunctional protective fabrics. In particular, the fabrics may be formed of high strength fibers that can be incorporated with other materials to produce comfortable garments and accessories that are resistant to abrasion, penetration, laceration, impact and are thermal and flame resistant.

Textile constructed using a double-knit modified interlock construction. Double knitting is a process by which two strands of yarn of the same or different varieties are knitted simultaneously on one pair of needles. The fabrics may be inseparable, as in interlock knitted fabrics, or they can simply be two unconnected textiles. A double knit interlock will create a fabric that has a tight ribbed appearance on both sides. These fabrics show good dimensional stability and are easy to cut and sew. They do not require any seam finishes as the fabric does not ravel. They are firm, stout, have low stretch and remain very resilient, making them an ideal candidate when designing durable textiles.

## Textile Products

Textile applications include those within the field of the DoD, industrial safety, public safety, medical and action sports markets. Products include—high wear areas in apparel, bags (particularly dry bags), inflatable boats, air bags, footwear (penetration resistant insoles for boots, booties, flip flops or for high abrasion areas on exterior), gloves, dive gear, etc. The invention also contemplates that a wide variety of garments and accessories may be manufactured from the trauma-resistant fabric, including but not limited to, wetsuits, drysuits, uniforms, vests, flight suits, pullovers, rash guards, jackets, coveralls, gear bags, pouches, pockets, harnesses, webgear, hats, helmets, headgear, shoes, skate shoes, insoles, socks, booties, cuffs, armbands, gloves, tents, armor, carriers, belts, bags, covers, rope and other items.

Without limiting the invention, the yarn may in some embodiments contemplate the use of additional fibers. Fibers contemplated herein include additional filaments being selected from the group consisting of: modified polyacrylonitrile, polyacrylonitrile, rayon, nylon, aramid, olefins, carbon, glass, and polyethylene including ultra high molecular weight polyethylene (UHMWPE).

Without limiting the invention, the yarn may in some embodiments contemplate the use of additional embedded materials or coatings. Embedded materials and coatings

contemplated herein include anti-bacterial coatings, silver coating, silver particles, silver nano particles, copper coating, copper particles, copper nano particles, as well as salts, conjugates, and combinations thereof.

In another embodiment, the invention contemplates the yarns may include, or be used in combination with, spun yarns, twisted yarns, plaited (braided) yarns, chopped yarns, filament yarns, jet blown yarns, core-wrapped yarns, and combinations thereof.

Weave patterns are also contemplated as within the scope of the inventive fabrics. Non-limiting preferred weave patterns include plain weave (alternating under/over of two perpendicular textile directions), plain dutch, reverse plain dutch, a 2x2 or 4x4 twill, twilled dutch, reverse twilled dutch, mesh, 3D-mesh, solid mesh, roll calendared, a unidirectional weave, a satin (periodic, e.g. 1-4, 1-5, or 1-8 under/over of perpendicular strands), crowfoot satin, herringbone, basket, sateen, diamond, percale, and honeycomb.

Referring now to FIG. 12, a variety of weave patterns are contemplated as within the scope of the invention, including without limitation, the plain weave, twilled weave, dutch plain weave, and dutch twilled weave, shown.

Referring to FIG. 13, FIG. 13 is a photomicrograph of 12 different types of weave patterns. For polymer fibers, various weave patterns are contemplated as within the scope of the invention, including without limitation, the plain weave, the plain dutch, the super mesh, the twilled 2-2 square, the twilled dutch, the reverse twilled dutch, the twilled 2-2 oblong, the reverse plain dutch, the roll calendared, the 3D mesh, the solid mesh, and the satin 1-4, shown.

Referring now to FIG. 18, there is a non-limiting example of a process for making the yarn and textiles described herein. Specifically, FIG. 18 shows a method of manufacturing a yarn for a textile, comprising the steps: (i) heating a multi-layer knitted textile in the presence of one or more dye compounds, wherein the multilayer knitted textile comprises a fabric outer layer and a fabric inner layer, wherein the fabric outer layer is knit from a first yarn containing a combination of modacrylic fibers and cotton fibers, wherein the fabric inner layer is knit from a second yarn made from 50-90% HBA/HNA filaments, wherein the heating shrinks the outer layer from about 5 to 25% in length, width, or both; (ii) assembling the multilayer knitted textile into an article; and (iii) performing a second heating of the article, wherein the second heating further shrinks the outer layer from about 2-10% in length, width, or both.

Referring now to FIG. 19 is a non-limiting illustration of the feature of a double heat-treated protective article, having a heat-treated multilayer knitted textile, according to the present invention. FIG. 19 shows that a double heat-treated protective article, having a heat-treated multilayer knitted textile, the heat-treated multilayer knitted textile comprising a fabric outer layer and a fabric inner layer, wherein the fabric outer layer is knit from a first yarn containing a combination of modacrylic fibers and cotton fibers, wherein the fabric inner layer is knit from a second yarn made from 50-90% HBA/HNA filaments, wherein the liquid crystal polymer filaments comprise a denier selected from the group consisting of 200d, 400d, 750d, 1000d, 1420d, 1500d, and 2250d, wherein the liquid crystal polymer filaments are melt spun fibers of a polycondensate of 4-hydroxybenzoic acid (HBA) and 6-hydroxynaphthalene-2-carboxylic acid (HNA) monomers (HBA/HNA), wherein the knit of the fabric inner layer is oriented at an oblique angle to the knit of the fabric outer layer, wherein the fabric outer layer is attached to the fabric inner layer, wherein the heat-treated multilayer knit-

ted textile is pre-shrunk about 10-15%, and wherein the protective article is secondarily heat-shrunk an additional 4%.

Referring now to FIG. 20, there is a non-limiting illustration of the two layer fabric, with a first layer having, e.g. cotton and modacrylic, and the second layer having a liquid crystal polymer knit fabric.

Referring now to FIG. 21, there is a non-limiting illustration of the heating and dyeing process of the two layer fabric, with a first layer having, e.g. cotton and modacrylic, having a wider knit, smaller number of loops per inch, before heating, and having a tighter, narrower knit, a greater number of loops per inch, after the heating. Since LCP textiles are difficult to dye, the addition of the first layer provides a (two-layer) dyed textile having the strength, puncture-resistance, cut-resistance, chemical resistance, and light weight characteristics of the underlying LCP textile while having the colorability, soft-feel, and fire-resistance of the modacrylic/blend. Additionally, the heat shrinkage, and increase in loop density, of the first layer, is joined by a parallel increase in loop density of the second layer since the two layer are attached, e.g. quilter, together. The shrinkage of the first layer causing an increased tightness of knit in the second layer adds a significant degree of strength and enhanced performance characteristics to the second LCP layer.

The references recited herein are incorporated herein in their entirety, particularly as they relate to teaching the level of ordinary skill in this art and for any disclosure necessary for the commoner understanding of the subject matter of the claimed invention. It will be clear to a person of ordinary skill in the art that the above embodiments may be altered or that insubstantial changes may be made without departing from the scope of the invention. Accordingly, the scope of the invention is determined by the scope of the following claims and their equitable Equivalents.

The invention claimed is:

1. A process for manufacturing a multilayer knitted textile, comprising the step of (i) heating a multi-layer knitted textile in the presence of one or more dye compounds at a temperature from 140-350 degrees F., wherein the multilayer knitted textile comprises a fabric outer layer and a fabric inner layer, wherein the fabric outer layer is knit from a first yarn containing a combination of modacrylic fibers and cotton fibers, wherein the fabric inner layer is knit from a second yarn made from 50-90% 4-hydroxybenzoic acid (HBA) and 6-hydroxynaphthalene-2-carboxylic acid (HNA) filaments, wherein the heating shrinks the outer layer from about 5 to 25% in length, width, or both.

2. The process of claim 1, wherein the first yarn includes one or more fibers selected from the group consisting of flame retardant (FR) rayon fibers, Opan fibers, and aramid fibers.

3. The process of claim 1, wherein the fabric outer layer is knit having a wale ranging from 17-27 loops per vertical inch and a course ranging from 18-24 loops per horizontal inch, and wherein after heating, the knit in loops per inch of the fabric outer layer is increased by about 15%.

4. The process of claim 1, wherein the fabric inner layer is attached to the fabric outer layer, and the shrinking of the fabric outer layer tightens the knit of the second yarn of the fabric inner layer.

5. The process of claim 1, wherein the heating shrinks the outer layer from about 10 to 20% in length, width, or both.

6. The process of claim 1, wherein the heating shrinks the outer layer about 15% in length, width, or both.

19

7. The process of claim 1, comprising the additional steps in order:

- (ii) assembling the multilayer knitted textile into an article; and
- (iii) performing a second heating of the article at a temperature of about 400 degrees F., wherein the second heating further shrinks the outer layer from about 2-10% in length, width, or both.

8. The process of claim 7, wherein the second heating further shrinks the outer layer about 4% in length, width, or both.

9. The process of claim 7, wherein the article is selected from the group of products consisting of apparel, bags, dry bags, inflatable boats, air bags, footwear, insoles for boots, booties, flip flops, gloves, dive gear, wetsuits, drysuits, uniforms, vests, flight suits, pullovers, rash guards, jackets, coveralls, shirts, trousers, gear bags, pouches, pockets, harnesses, web-gear, hats, helmets, headgear, shoes, skate shoes, insoles, socks, cuffs, armbands, gloves, tents, armor, carriers, belts, bags, covers, furnishings, drapery, outdoor fabric, and rope.

10. The process of claim 7, wherein the article is selected from the group of products consisting of apparel, bags, dry bags, inflatable boats, air bags, footwear, insoles for boots, booties, flip flops, gloves, dive gear, wetsuits, drysuits, uniforms, vests, flight suits, pullovers, rash guards, jackets, coveralls, shirts, trousers, gear bags, pouches, pockets, harnesses, web-gear, hats, helmets, headgear, shoes, skate shoes, insoles, socks, cuffs, armbands, gloves, tents, armor, carriers, belts, bags, covers, furnishings, drapery, outdoor fabric, and rope.

11. The process of claim 1, wherein the HBA/HNA filaments comprise a denier selected from the group consisting of 200d, 400d, 750d, 1000d, 1420d, 1500d, and 2250d.

12. The process of claim 1, wherein the HBA/HNA filaments are melt spun fibers of a polycondensate of 4-hydroxybenzoic acid (HBA) and 6-hydroxynaphthalene-2-carboxylic acid (HNA) monomers (HBA/HNA).

13. The process of claim 1, wherein the multilayer textile comprises at least one additional fabric layer.

14. The process of claim 1, wherein the fabric inner layer is attached to the fabric outer layer using a knitting technique, is sewn, is interlock knitted to, or is plaited with the fabric outer layer as an overbraid.

15. The process of claim 1, wherein the knit of the fabric inner layer is oriented at an oblique angle to the knit of the fabric outer layer.

20

16. The process of claim 1, wherein the knit of the fabric inner layer is oriented at an orthogonal angle to the knit of the fabric outer layer.

17. The process of claim 1, wherein the one or dyes are disperse dyes selected from the group consisting of: Nitro Dyes, Amino Ketone dyes, Anthraquinonoid dyes, Mono azo dyes, Di-azo dyes, and mixtures thereof.

18. The process of claim 17, wherein the disperse dyes are applied using a method selected from the group consisting of: Normal dyeing method at a Dyeing temperature 80-100° C., a Normal Method of dyeing with carriers at a Dyeing temperature 80-100° C., a High temperature dyeing method at a Dyeing temperature 105-140° C., a Thermasol dyeing method at a Dyeing temperature 180-220° C., a Semi continuous Pad roll dyeing method, and a Continuous Pad steam method.

19. A double heat-treated protective article, having a heat-treated multilayer knitted textile, the heat-treated multilayer knitted textile comprising a fabric outer layer and a fabric inner layer, wherein the fabric outer layer is knit from a first yarn containing a combination of modacrylic fibers and cotton fibers, wherein the fabric inner layer is knit from a second yarn made from 50-90% HBA/HNA filaments, wherein the liquid crystal polymer filaments comprise a denier selected from the group consisting of 200d, 400d, 750d, 1000d, 1420d, 1500d, and 2250d, wherein the liquid crystal polymer filaments are melt spun fibers of a polycondensate of 4-hydroxybenzoic acid (HBA) and 6-hydroxynaphthalene-2-carboxylic acid (HNA) monomers (HBA/HNA), wherein the knit of the fabric inner layer is oriented at an oblique angle to the knit of the fabric outer layer, wherein the fabric outer layer is attached to the fabric inner layer, wherein the heat-treated multilayer knitted textile is pre-shrunk about 10-15%, and wherein the protective article is secondarily heat-shrunk an additional 4%.

20. The article of claim 19, wherein the article is selected from the group of products consisting of apparel, bags, dry bags, inflatable boats, air bags, footwear, insoles for boots, booties, flip flops, gloves, dive gear, wetsuits, drysuits, uniforms, vests, flight suits, pullovers, rash guards, jackets, coveralls, shirts, trousers, gear bags, pouches, pockets, harnesses, web-gear, hats, helmets, headgear, shoes, skate shoes, insoles, socks, cuffs, armbands, gloves, tents, armor, carriers, belts, bags, covers, furnishings, drapery, outdoor fabric, and rope.

\* \* \* \* \*